

## UNITED STATES PATENT OFFICE

ADOLPH A. PRUSSIN, OF NEW YORK, N. Y., ASSIGNEE TO PETRO-SOL CORPORATION, A CORPORATION OF DELAWARE

## PROCESS FOR THE SOLIDIFICATION OF LIQUID HYDROCARBONS

No Drawing.

Application filed November 20, 1930. Serial No. 497,056.

My invention relates to a new and useful process of solidification of liquid hydrocarbons.

The process can be applied to the solidification of kerosene, naphtha, gasoline, benzol, lubricating oil, fuel oil, gas oil, crude oil and other liquid hydrocarbons. When any of the said hydrocarbons is solidified it is an entirely new product containing the hydrocarbon which has been solidified.

The objects of my invention are as follows;

1.—To produce a solid made from a liquid hydrocarbon.

15 2.—To eliminate the explosiveness and high inflammability of light hydrocarbons in use, in storage and in transportation.

3.—To minimize the evaporation losses in handling hydrocarbons.

20 4.—To reduce hydrocarbons to solid products so as to change them into the state from which greatest efficiency can be obtained in use for motive power, for fuel and for light.

Other objects will appear as set forth in the descriptive matter herein.

The process consists of adding to the liquid hydrocarbon  $1\frac{1}{2}\%$  by volume of albumin, bringing this mixture to a temperature of 104 degrees Fahrenheit, then cooling the mixture and adding 2% by volume of acetone, thus causing a precipitate, removing the precipitate by decantation or other means, then heating the hydrocarbon, to a temperature of about 150 degrees Fahrenheit, at which point solidification takes place.

## Example:—

1. Mix.

Kerosene-----  $96\frac{1}{2}$  parts  
Albumen-----  $1\frac{1}{2}$  "

40 2. Heat to 104 degrees F.

3. Allow to cool.

4. Add.

Acetone----- 2 "

45 5. Remove precipitation.  
6. Heat to 150 degrees F.

## What I claim is

1. A process of solidification of liquid hydrocarbons consisting in mixing by volume 50  $96\frac{1}{2}$  parts of liquid hydrocarbon with  $1\frac{1}{2}$

parts of albumin, heating said mixture to a moderate temperature, cooling, adding to the mixture 2 parts of acetone, removing the precipitated albumin and solidifying the liquid hydrocarbon by moderate heat.

55

2. A process of solidification of liquid hydrocarbons consisting in the mixing by volume  $96\frac{1}{2}$  parts of liquid hydrocarbon with  $1\frac{1}{2}$  parts of albumin, heating said mixture to a temperature of about 104 degrees, Fahrenheit, cooling, adding to the mixture 2 parts of acetone, removing the precipitated albumin and solidifying the liquid hydrocarbon by heating to about 140 degrees, Fahrenheit.

60

Signed at New York City in the county of New York and State of New York this 10th day of November A. D. 1930.

ADOLPH A. PRUSSIN.

65